# EUROPEAN PATENT APPLICATION

(11) **EP 2 284 246 A1**
(43) Date of publication of application: **16.02.2011**
(21) Application number: 10169196.2
(22) Date of filing: 12.07.2010
(51) Int. Cl.: C10M 103/02, C10N 30/06, C10N 40/12

(54) **Coating for turbomachinery**

(30) Priority: 17.07.2009 US 504837
(71) Applicant: General Electric Company, Schenectady, NY 12345 (US)
(72) Inventor: Bucci, David Vincent, Simpsonville, SC 29681 (US); Dimascio, Paul Stephen, Greer, SC 29650 (US); Pabla, Surinder S., Greer, SC 29650 (US); Moses, Jesse C., Greenville, SC 29611 (US)
(74) Representative: Szary, Anne Catherine

(57) **Abstract**

A coating for turbomachinery comprises graphite-based solid film lubricant material.

## Description

### BACKGROUND OF THE INVENTION

The invention is directed to surface treatments for rotating turbomachinery. In particular, the invention is directed to surface treatments for gas turbine components that may exhibit stresses, and in further particularity, the invention is directed to surface treatments for gas turbine compressor blade components at their interface with compressor wheels, where they may exhibit stresses.

Previous gas turbine compressor blade component configuration may provide bare or non-treated compressor blades with an interface at the compressor wheel. For example, the compressor blade of the compressor may contact, or define an interface, against compressor wheels, such as but not limited to, CrMoV wheels. These areas of contact are at areas of high contact stresses between the elements. These stresses can lead to undesirable effects, such as but not limited to, fretting and galling. These undesirable effects, if left unaddressed, may lead to component failures and possible shutdown of related gas turbine units.

### BRIEF DESCRIPTION OF THE INVENTION

According to an aspect of the invention, a coating for turbomachinery comprises graphite-based solid film lubricant material.

In another aspect of the invention, a coating for turbomachinery is provided and comprises graphite-based solid film lubricant material; where the turbomachinery comprises at least a wheel comprising a slot and a bucket comprising a dovetail, the coating is applied to at least one of the slot and the dovetail; and coating comprises at least one of: graphite-based dry film lubricants, metal filled resin based systems, silicate binder with graphite; and high temperature lubricating additives.

Further, in yet another non-limiting aspect of the invention, A method for coating for turbomachinery to provide at least one of crevice corrosion resistance and fretting resistance, the method comprising providing a coating; and applying the coating to at least one of the slot and the dovetail; wherein the coating comprises graphite-based solid film lubricant material; the turbomachinery comprises at least a wheel comprising a slot and a bucket comprising a dovetail, the coating is applied to; and the coating comprises at least one of graphite-based dry film lubricants, metal filled resin based systems, silicate binder with graphite; and high temperature lubricating additives.

### BRIEF DESCRIPTION OF THE DRAWINGS

These and other features, aspects, and advantages of the present invention will become better understood when the following detailed description is read with reference to the accompanying drawings, by way of example, in which like characters represent like parts throughout the drawings, wherein:

FIG. 1 is a perspective view of a portion of a turbine or compressor disc employing balancing apparatus, as embodied by the invention;

FIG. 2 is a detailed side view of a portion of two adjacent compressor states, as embodied by the invention, which permits the radial insertion of balance weights after assembly of the adjacent stages; and

FIG. 3 is a further side view of a portion of two adjacent compressor states, as embodied by the invention, which permits the radial insertion of balance weights after assembly of the adjacent stages.

### DETAILED DESCRIPTION OF THE INVENTION

Although the present invention may have general application to both turbomachinery, such as but not limited to, turbine wheels and compressor wheels, particularly for gas or steam turbines, the following embodiment is directed toward a compressor stage of a gas or steam turbine for concreteness of description. This description is not intended to limit the invention in any manner.

A compressor stage is conventionally fabricated with a wheel or disc affixed or integrally formed with an axial shaft. Female dovetail regions are machined into the surface of the wheel and male dovetail regions of compressor blades are fitted into the female dovetails.

Illustrated in FIG. 1 is a portion of a compressor 10, for example, a compressor of a gas turbine engine. The compressor 10 includes an inlet; first stage bladed disk assembly 12 disposed upstream of and coaxially with a plurality of circumferentially spaced stator vanes 14 about an engine or compressor longitudinal centerline 16. The bladed disk assembly 12 includes a plurality of circumferentially spaced rotor blades 18 attached to a rotor wheel or disk 20.

More specifically, and referring to both FIGS. 1 and 2, the blade 18 includes a relatively thin, solid airfoil portion 22 having a tip 24, a root 26, a leading edge 28, and a trailing edge 30. The blade 18 further includes a generally rectangular platform 32 extending laterally outwardly from the airfoil root 26. The platform 32 is relatively highly sloped, upwardly toward the tip 24, from the leading edge 28 to the trailing edge 30, and provides an inner airflow boundary in the compressor 10. The platform 32 includes an upstream, forward end 34 and a downstream aft end 36, the aft end 36 being disposed at a radius greater than that of the forward end 34. The blade 18 also includes a shank 38 extending coaxially from the airfoil 22 at the platform 32, and a conventionally shaped axial entry dovetail 40 extending from the shank 38. Further, the blade 18 can be formed from any appropriate material, suitable for a turbine component blade. For example, and in no way limiting of the invention, the compressor blade can comprise at least one of graphite, graphite containing materials, and other such carbon fiber materials.

Further, as embodied by the invention, the blade 18 of the turbomachinery may be formed of a superalloy, such as a precipitation hardenable, nickel-based alloy (Inconnel 718), or from stainless steel materials.

The wheel or disk 20 includes a plurality of axially disposed circumferentially spaced slots 42 in an outer perimeter 44 thereof which are complementary in shape to the blade dovetails 40, and which receive the dovetails 40 for attaching the blades 18 thereto. Air 46 is suitably channeled through the blades 18 and the vanes 14 and is compressed thereby.

Contact stresses between the compressor blade dovetail 40 and wheel 20 combined with the movement of the part in the wheel slot 42 when the turbine rotor and bladed disk assembly 12 rotates. These contact stresses can lead to high contact stress fretting and galling wear of the bladed disk assembly 12. To reduce the friction coefficient at the contact surface and lower the wear rate therebetween, a coating 50, as embodied by the invention, is applied to at least one of the bladed disk assembly 12 and the slot 42.

Preferably, the coating 50 is applied to the bladed disk assembly 12 surfaces in the slot 42, as embodied by the invention; however, the coating 50 can be the wheel slot 42. A coating 50 can be applied to either or both adjacent surfaces, of the bladed disk assembly 12 and/or the slot 42.

Applying coatings to the materials that form the bladed disk assembly 12 and the wheel 20, such as materials comprising duplex stainless steel materials, can be difficult due to geometry of these components. For example, and in no way limiting of the invention, some coatings can cause crevice corrosion issues on such materials. Accordingly, as embodied by the invention, coatings 50, as embodied by the invention, comprise a graphite-based solid film lubricant coating. Further, the coating 50 can comprise at least one of graphite based dry film lubricants or metal filled resin based systems that can be applied to at least one of the bladed disk assembly 12 and the wheel slot 42. These coating materials, as embodied by the invention, can be used to lower friction coefficients and reduce wear between the bladed disk assembly 12 and the wheel slot 42.

The coating 50, as embodied by the invention, provides at least one of anti-fretting resistance and resistance to crevice corrosion.

The coating 50 may comprise graphite materials, and it is within the scope of the invention that the coating comprises graphite grease. Moreover, the coating 50, as embodied by the invention, may comprise molybdenum grease, either alone or in combination with other graphite-based solid film lubricant coating materials.

For example, materials for the coating, as embodied by the invention, include limited to products, such as but not limited to, lubricants; dry lubricants; lubricants and bonding materials in a suitable solvent, an oil-soluble; sulfonate surfactant/wetting agent (for example SurfKote® LOB-1800-G from HOHMAN PLATING & MFG. INC.); titanium containing lubricants, such as but not limited to, Alumazite ZDA (from Tiodize Co., Inc.) and combinations thereof. In general, the coatings comprise a lubricating material, which can be combined with other components that provide desired material characteristics. For example, one non-limiting coating material can comprise silicate binder with graphite and other high temperature lubricating additives. Other additives can be desired dependent on the intended use of the blade, the environment of the blade and associated turbomachinery.

The coating 50, as embodied by the invention, are preferably applied to a compressor blade dovetail 40 of the blade 18 where it contacts the wheel slot 42. However, as embodied by the invention, the coating 50 can be applied to any pressure face surfaces of the dovetail 40 and/or the slot 42, if needed.

The coating 50, as embodied by the invention, is applied at a thickness in range from about 0.0005" to about 0.002". The coating 50 can be applied at a thickness, which can prevent galling, seizing and fretting of the dovetail base metal/substrate.

The coating 50, as embodied by the invention, can be applied by any appropriate coating process. Further, Exemplary coating processes, include, but are not limited to, painting; deposition, such as but not limited to, physical vapor deposition, plasma-enhanced chemical vapor deposition, and chemical vapor deposition; sputtering, such as etching and chemical sputtering; powder coating; air plasma spray, cold spraying, electroplating; and combinations thereof.

In conventional turbomachinery, bare compressor blades pressing against wheels, such as but not limited to, wheels formed of CrMoV, at high contact stresses may lead to excessive fretting and galling, among other undesired effects. This excessive fretting and galling, which left unaddressed, has shown to lead to component faults and possible shutdowns of turbomachinery and gas turbine units. The coating on the blade dovetail, as embodied by the invention, is effective in reducing a wear thereon to extend the turbomachinery component's lifetime. This improvement may also lead to improved gas turbine and/or compressor reliability. Also, the coating of the blade, as embodied by the invention, is simpler, less expensive and a more robust process than attempting to coat turbomachinery in the hard to reach areas, such as but not limited to, wheel slots of the turbine wheel into which blades slide.

The blades with the coating, as embodied by the invention, provide an anti fretting coating solution that will not cause crevice corrosion. The coating 50, as embodied by the invention, can be applied and coat superalloy substrates, such as a GTD450 blade, which can be difficult since coatings on GTD450 experience crevice corrosion issues. The blades with the coating, as embodied by the invention, can run as designed with high contact stresses, which may occur as a result of the operation of the turbomachinery. Further, as embodied by the invention, the coated component should not fail with the same fallout rate in the un-coated version.

While only certain features of the invention have been illustrated and described herein, many modifications and changes will occur to those skilled in the art. It is, therefore, to be understood that the appended claims are intended to cover all such modifications and changes as fall within the true scope of the invention.

## Claims

1. A coating for turbomachinery, the coating comprising:
graphite-based solid film lubricant material.

2. The coating for turbomachinery according to claim 1, wherein the coating provides at least one of crevice corrosion resistance and fretting resistance.

3. The coating for turbomachinery according to claim 1 or claim 2, wherein the turbomachinery comprises at least a wheel comprising a slot and a bucket comprising a dovetail, and wherein the coating is applied to at least one of the slot and the dovetail.

4. The coating for turbomachinery according to claim 3, wherein the coating is applied to the dovetail.

5. The coating for turbomachinery according to any preceding claim, wherein the turbomachinery comprises a superalloy material.

6. The coating for turbomachinery according to any preceding claim, wherein the coating comprises graphite-based dry film lubricants.

7. The coating for turbomachinery according to any preceding claim, the coating comprises metal filled resin based systems.

8. The coating for turbomachinery according to any preceding claim, wherein the coating further comprises at least one of silicate binder with graphite and high temperature lubricating additives.

9. The coating for turbomachinery according to any preceding claim, the coating comprising:
graphite-based solid film lubricant material;
the turbomachinery comprises at least a wheel comprising a slot and a bucket comprising a dovetail, wherein the coating is applied to at least one of the slot and the dovetail;
and the coating comprises at least one of: graphite-based dry film lubricants, metal filled resin based systems, silicate binder with graphite; and high temperature lubricating additives.

10. The coating for turbomachinery according to claim 9, wherein the coating is applied to the dovetail.

11. The coating for turbomachinery according to claim 9 or claim 10, wherein the turbomachinery comprises a superalloy material.

12. The coating for turbomachinery according to any one of claims 9 to 11, wherein the coating provides at least one of crevice corrosion resistance and fretting resistance.

13. A method for coating for turbomachinery to provide at least one of crevice corrosion resistance and fretting resistance, the method comprising:
providing a coating; and
applying the coating to at least one of a slot and a dovetail; wherein the coating comprises: graphite-based sold film lubricant material; the turbomachinery comprises at least a wheel comprising a slot and a bucket comprising a dovetail, the coating is applied to; and the coating comprises at least one of graphite-based dry film lubricants, metal filled resin based systems, silicate binder with graphite; and high temperature lubricating additives.
